



greater detail in "Introduction to Organic Chemistry," Condon & Meislich, Holt, Rinehart & Winston, Inc., New York (1961).

### ACETYLENIC ALCOHOLS

The acetylenic alcohols include those alcohols containing the acetylenic grouping and contain from 3-12 carbon atoms. The preferred alcohols used in the practices of this invention are propargyl alcohol and, most preferably, 4-ethyl-1-octyn-3-ol. Other alcohols suitable for use in preparing the compositions of the invention come within the following structural formula:



wherein R is —H, alkyl or phenyl and R' is —H or lower alkyl.

Alcohols of the above type are set forth in U.S. 3,049,496, the disclosure of which is incorporated herein by reference.

### THE OIL SOLUBLE DISPERSANTS

The oil soluble dispersants used in preparing finished inhibitor products are most preferably oil soluble or at least oil dispersible. They are either anionic or non-ionic at use levels. The non-ionic products are prepared by reacting fatty acids, alcohols, alkyl phenols and the like with between 5-50 moles of either ethylene or propylene oxide.

Preferred chemicals of this type are the alkyl phenols or fatty acids which have been reacted with from between 5-25 moles of ethylene oxide.

Fatty acids per se, e.g. C12-C22 fatty acids, may be used as well as the polymerized diethanoid fatty acids which form dimers and trimers and mixtures thereof upon polymerization. See particularly U.S. 2,482,761 and 2,763,612. When the fatty acids are used alone it is desirable that they be used as the free acid rather than as their soaps or salts.

The oil soluble dispersants of the types described above when used in preparing corrosion inhibiting compositions tend to improve the operability of the Mannich reaction products in combination with the acetylenic alcohol. They allow the alcohol, particularly the higher alcohols, to be dissolved or dispersed into the mineral acid. They perform a similar function with respect to Mannich reaction products. They are also important in that they provide a better wetting of the inhibitor on the metal surfaces sought to be protected.

### THE ORGANIC SOLVENTS

Many of the well-known organic solvents can be used to dissolve the above-described ingredients. Preferably these solvents are petroleum base solvents and contain at least 20% by weight of aromatic constituents. Thus, such well-known fractions as aromatic oils, Stoddard solvents, naphthas and the like may be utilized. Generally those aromatic solvents having a boiling point above that of gasoline but below that of lubricating oils are satisfactory.

Other well-known organic solvents that may be used are for instance, benzene, toluene, xylene, dimethylformamide, dimethylsulfoxide and the like.

### THE EVALUATION OF THE INVENTION

Listed below are typical compositions of the invention; Compositions I through III and IX and X are Mannich reaction products.

### EXAMPLE I

#### Composition 1

|   |                            | Gms. |
|---|----------------------------|------|
| 5 | Rosin amine D <sup>1</sup> | 90   |
|   | Muriatic acid (30% HCl)    | 30   |
|   | Isopropanol (99%)          | 100  |
|   | Formalin (37%)             | 80   |
|   | Acetaldehyde               | 88   |

10 <sup>1</sup> Hydroabietyl amine.

The above were added to a three necked flask and heated between 60° and 70° C. for 4 hours to yield the finished product.

### EXAMPLE II

#### Composition 2

|    |                            | Gms. |
|----|----------------------------|------|
| 20 | Rosin amine D <sup>1</sup> | 17   |
|    | Muriatic acid              | 6    |
|    | Isopropanol (99%)          | 50   |
|    | Formalin (37%)             | 8    |
|    | Acetaldehyde               | 9    |

1 Hydroabietyl amine.

25 The above were added together to a Fisher Pressure bottle in the order listed, sealed and mounted on a revolving wheel at 160° F. for 16 hours.

### EXAMPLE III

#### Composition 3

|    |                            | Gms. |
|----|----------------------------|------|
| 30 | Rosin amine D <sup>1</sup> | 9    |
|    | Muriatic acid              | 3    |
|    | Isopropanol                | 50   |
|    | Formalin (37%)             | 8    |
|    | Acetaldehyde               | 9    |

1 Hydroabietyl amine.

40 The above were added together to a Fisher Pressure bottle and mounted on the wheel for 24 hours at 160° F.

#### Composition 4

|    |                                      | Gms. |
|----|--------------------------------------|------|
| 45 | Composition 2                        | 20   |
|    | Nonyl phenol+12 moles ethylene oxide | 30   |
|    | Crude tall oil                       | 20   |
|    | Propargyl alcohol                    | 10   |

#### Composition 5

|    |                                      |    |
|----|--------------------------------------|----|
| 50 | Composition 3                        | 40 |
|    | Nonyl phenol+12 moles ethylene oxide | 20 |
|    | Crude tall oil                       | 30 |
|    | Propargyl alcohol                    | 10 |

#### Composition 6

|    |                                      |    |
|----|--------------------------------------|----|
| 55 | Composition 2                        | 20 |
|    | Nonyl phenol+12 moles ethylene oxide | 15 |
|    | Tall oil+15 moles ethylene oxide     | 15 |
|    | Crude tall oil                       | 40 |
|    | Propargyl alcohol                    | 10 |

#### Composition 7

|    |                                      |    |
|----|--------------------------------------|----|
| 60 | Composition 2                        | 30 |
|    | Nonyl phenol+12 moles ethylene oxide | 15 |
|    | Tall oil+15 moles ethylene oxide     | 15 |
|    | Crude tall oil                       | 30 |
|    | Propargyl alcohol                    | 10 |

#### Composition 8

|    |                                      |    |
|----|--------------------------------------|----|
| 70 | Composition 2                        | 12 |
|    | Nonyl phenol+12 moles ethylene oxide | 7  |
|    | Tall oil+15 moles ethylene oxide     | 8  |
|    | Crude tall oil                       | 20 |
|    | Propargyl alcohol                    | 2  |

## 5

## EXAMPLE IV

## Composition 9

|                            | Gms. |
|----------------------------|------|
| Rosin amine D <sup>1</sup> | 51   |
| Muriatic acid              | 18   |
| Isopropanol (99%)          | 25   |
| Formalin (37%)             | 24   |
| Acetaldehyde               | 27   |

<sup>1</sup> Hydroabietyl amine.

The above was added to a Fisher Pressure bottle and mounted on a revolving wheel at 160° F. for 72 hours.

## EXAMPLE V

## Composition 10

|                            | Gms. |
|----------------------------|------|
| Rosin amine D <sup>1</sup> | 34   |
| Muriatic acid              | 12   |
| Isopropanol (99%)          | 25   |
| Formalin (37%)             | 40   |
| Acetaldehyde               | 40   |

<sup>1</sup> Hydroabietyl amine.

The above were added to a Fisher Pressure bottle and mounted on the wheel for 72 hours.

## Composition 11

|                   | Gms. |
|-------------------|------|
| Composition 9     | 67   |
| Isopropanol (99%) | 62   |

## Composition 12

|                                      | Gms. |
|--------------------------------------|------|
| Composition 11                       | 30   |
| Aromatic solvent                     | 50   |
| Octynol <sup>2</sup>                 | 10   |
| Nonyl phenol+12 moles ethylene oxide | 10   |

<sup>2</sup> 4-ethyl-1-octyn-3-ol.

## Composition 13

|                                      | Gms. |
|--------------------------------------|------|
| Composition 11                       | 20   |
| Tall oil+15 moles ethylene oxide     | 15   |
| Nonyl phenol+12 moles ethylene oxide | 15   |
| Crude tall oil                       | 20   |
| Aromatic solvent                     | 20   |
| Octynol <sup>2</sup>                 | 10   |

<sup>2</sup> 4-ethyl-1-octyn-3-ol.

## Composition 14

|                   | Gms. |
|-------------------|------|
| Composition 13    | 80   |
| Polyamine bottoms | 20   |

## Composition 15

|                                            | Gms. |
|--------------------------------------------|------|
| Composition 13                             | 80   |
| Dimer and trimer fatty acids-still bottoms | 20   |

## Composition 16

|                     | Gms. |
|---------------------|------|
| Composition 13      | 80   |
| Sulfurized tall oil | 20   |

## Composition 17

|                | Gms. |
|----------------|------|
| Composition 13 | 80   |
| KI             | 4    |
| Water          | 16   |

## Composition 18

|                                            | Gms. |
|--------------------------------------------|------|
| Composition 13                             | 80   |
| Dimer and trimer fatty acids-still bottoms | 20   |

## 6

## Composition 19

|                                      | Gms. |
|--------------------------------------|------|
| Composition 11                       | 20   |
| Nonyl phenol+12 moles ethylene oxide | 15   |
| 5 Tall oil+15 moles ethylene oxide   | 15   |
| Aromatic solvent                     | 40   |
| Octynol <sup>2</sup>                 | 5    |
| Aromatic solvent                     | 15   |

<sup>2</sup> 4-ethyl-1-octyn-3-ol.

10

## Composition 20

|                                         | Gms. |
|-----------------------------------------|------|
| Composition 11                          | 30   |
| Aromatic solvent                        | 50   |
| Octynol <sup>2</sup>                    | 10   |
| 15 Nonyl phenol+12 moles ethylene oxide | 10   |

<sup>2</sup> 4-ethyl-1-octyn-3-ol.

## Composition 21

|                                      | Gms. |
|--------------------------------------|------|
| 20 Composition 9                     | 20   |
| Nonyl phenol+12 moles ethylene oxide | 15   |
| Tall oil+15 moles ethylene oxide     | 15   |
| Crude tall oil                       | 20   |
| Aromatic solvent                     | 20   |
| Octynol <sup>2</sup>                 | 10   |

<sup>2</sup> 4-ethyl-1-octyn-3-ol.

## Composition 22

|                                      | Gms. |
|--------------------------------------|------|
| 30 Composition 9                     | 10   |
| Tall oil+15 moles ethylene oxides    | 25   |
| Nonyl phenol+12 moles ethylene oxide | 15   |
| Crude tall oil                       | 20   |
| Aromatic solvent                     | 20   |
| Octynol <sup>2</sup>                 | 10   |

<sup>2</sup> 4-ethyl-1-octyn-3-ol.

## Composition 23

|                   | Gms. |
|-------------------|------|
| 40 Composition 13 | 90   |
| KI                | 5    |
| Water             | 5    |

## Composition 24

|                   | Gms. |
|-------------------|------|
| 45 Composition 13 | 80   |
| KI                | 10   |
| Water             | 10   |

## Composition 27

|                                                                   | Gms. |
|-------------------------------------------------------------------|------|
| 50 Composition 13                                                 | 45   |
| Hydroabietyl amines+5 moles ethylene oxide+15% hydroabietyl amine | 5    |

## CORROSION TESTS

In the small scale laboratory tests which follow, three different types of ferrous metal specimens were used:

## Specimens

(1) High pressure steel tubing—American Petroleum Institute designation N-80.

(2) Mild steel coupons SAE 1020 cold rolled steel.

(3) High carbon steel drill rod.

All tests used 15% HCl solutions as the test media.

No blank results are indicated since under the test conditions at temperatures in excess of 150° the test specimens were completely destroyed.

In a series of tests corresponding to those hereinafter described the Mannich reaction products were evaluated and were found to be no better than the blank test results.

4-ethyl-1-octyn-3-ol was evaluated under the test conditions shown and the concentrations used in the test and in all instances gave 50% poorer results than the compositions of the invention.

Results of testing the various compositions of the invention are set forth below in Table I.

TABLE I

| Test No. | Comp. No. | Time, hrs. | Temp., °F. | Specimen type | Cone., gal. 1,000 | Wt. loss, g. |
|----------|-----------|------------|------------|---------------|-------------------|--------------|
| 1        | 4         | 6          | 200        | 1             | 4                 | 3.0062       |
| 2        | 5         | 6          | 200        | 1             | 4                 | 2.9763       |
| 3        | 4         | 6          | 200        | 1             | 2                 | 4.5123       |
| 4        | 4         | 6          | 200        | 1             | 2                 | 5.2470       |
| 5        | 6         | 6          | 200        | 1             | 4                 | 0.5123       |
| 6        | 7         | 5½         | 200        | 1             | 2                 | 2.8084       |
| 7        | 7         | 5½         | 200        | 1             | 4                 | 0.5458       |
| 8        | 8         | 5½         | 200        | 1             | 2                 | 1.4868       |
| 9        | 8         | 5½         | 200        | 1             | 4                 | 1.2646       |
| 10       | 6         | 24         | 200        | 1             | 2                 | 20.7465      |
| 11       | 6         | 24         | 200        | 1             | 4                 | 1.5616       |
| 12       | 14        | 6          | 200        | 3             | 4                 | 1.48.9       |
| 13       | 16        | 6          | 200        | 3             | 4                 | 1.47.9       |
| 14       | 17        | 6          | 200        | 3             | 4                 | 1.60.5       |
| 15       | 18        | 6          | 200        | 3             | 4                 | 1.76.6       |
| 16       | 13        | 6          | 200        | 3             | 4                 | 1.60.4       |
| 17       | 19        | 6          | 200        | 3             | 4                 | 1.61.1       |
| 18       | 20        | 6          | 200        | 3             | 4                 | 1.67.7       |
| 19       | 21        | 8          | 200        | 3             | 4                 | 1.76.4       |
| 20       | 22        | 8          | 200        | 3             | 4                 | 1.44.9       |
| 21       | 13        | 8          | 200        | 3             | 4                 | 1.37.5       |
| 22       | 13        | 18         | 200        | 3             | 2                 | 1.15.4       |
| 23       | 23        | 18         | 200        | 3             | 1                 | 1.79.0       |
| 24       | 23        | 18         | 200        | 3             | 2                 | 1.13.9       |
| 25       | 24        | 18         | 200        | 3             | 1                 | 1.62.1       |
| 26       | 24        | 18         | 200        | 3             | 2                 | 1.11.5       |
| 27       | 28        | 5          | 200        | 3             | 4                 | 1.35.9       |
| 28       | 7         | 24         | 72         | 2             | 1                 | 10.2047      |
| 29       | 7         | 24         | 72         | 2             | 2                 | 1.1672       |

<sup>1</sup> In milligrams.

## CONCLUSION

While the tests have shown the compositions to be effective in inhibiting 15% hydrochloric acid, they are also effective in inhibiting the various strength hydrochloric acid solutions up to its saturation solubility. They are similarly effective in inhibiting solutions of phosphoric, sulfuric and nitric acids.

What is claimed is:

1. An aqueous solution substantially non-corrosive to ferrous metals which consists essentially of a major proportion of an inorganic mineral acid from the group consisting of hydrochloric, phosphoric, sulfuric, and nitric acid and from 0.001 to 2% by volume of a composition consisting essentially of:

(A) the Mannich reaction condensation product of one mole of a hydroabietyl amine with at least two moles of formaldehyde and at least two moles of an aldehyde containing from 2 to 6 carbon atoms and having at least one hydrogen atom on the carbon atom adjacent to the aldehydic carbonyl carbon atom, and

(B) a monohydroxy acetylenic alcohol which contains from 3 to 12 carbon atoms: with the ratio of A to B being within the range of from 5:1 to 1:5.

2. The aqueous solution of an inorganic mineral acid as set forth in claim 1 where the mineral acid is hydrochloric.

3. The aqueous solution of an inorganic mineral acid as set forth in claim 1 wherein R' and A are hydrogen and the acetylenic alcohol is 4-ethyl-1-octyn-3-ol.

4. The aqueous solution of an inorganic mineral acid as set forth in claim 3 wherein the ratio of A to B is within the range of from 3:1 to 1:3.

5. The aqueous solution of an inorganic mineral acid as set forth in claim 4 wherein the ratio of A to B is within the range of 1:1 to 1:3.

6. A composition useful in inhibiting the corrosive tendencies of aqueous solutions of inorganic mineral acids from the group consisting of hydrochloric, phosphoric, sulfuric, and nitric acid, which consists essentially of from 10% to 30% by weight of a composition consisting essentially of:

(A) the Mannich reaction condensation product of one mole of hydroabietyl amine with at least two moles of formaldehyde and at least two moles of an aldehyde containing from 2 to 6 carbon atoms and having at least one hydrogen atom on the carbon atom adjacent to the aldehydic carbonyl carbon atom, and

(B) a monohydroxy acetylenic alcohol which contains from 3 to 12 carbon atoms;

20 with the ratio of A to B being within the range of from 5:1 to 1:5, 5-40% by weight of an oil soluble dispersant formed by reacting higher fatty acids and higher alkyl phenols with 5-50 moles of an alkoxide from the group consisting of ethylene oxide and propylene oxide; the balance being a hydrocarbon solvent for the above ingredients having a boiling point above 75° C.

25 7. The composition of claim 6 wherein R' and A are hydrogen and the acetylenic alcohol is 4-ethyl-1-octyn-3-ol; and wherein the oil soluble dispersant is an ethoxylated nonyl substituted phenol which contains from 5-50 moles of reacted ethylene oxide.

## References Cited

## UNITED STATES PATENTS

|           |         |                        |             |
|-----------|---------|------------------------|-------------|
| 2,975,125 | 3/1961  | Saukaitis et al. ----- | 252—8.55    |
| 3,077,454 | 2/1963  | Monroe et al. --       | 252—8.55 CX |
| 3,107,221 | 10/1963 | Harrison et al. -----  | 252—148     |
| 3,113,113 | 12/1963 | Marsh et al. -----     | 252—392     |
| 3,230,173 | 1/1966  | Spivack -----          | 252—148     |
| 3,249,548 | 5/1966  | Herman et al. ----     | 252—146X    |

MAYER WEINBLATT, Primary Examiner

A. I. RADY, Assistant Examiner

U.S. Cl. X.R.

252—146, 148, 392; 260—584

UNITED STATES PATENT OFFICE  
CERTIFICATE OF CORRECTIONPatent No. 3,585,136 Dated June 15, 1971Inventor(s) James R. Stanford et al

It is certified that error appears in the above-identified patent and that said Letters Patent are hereby corrected as shown below:

Column 5, Composition 12 should read as follows:

|                                           | Gms. |
|-------------------------------------------|------|
| Composition 11 -----                      | 20   |
| Nonyl phenol+12 moles ethylene oxide----- | 15   |
| Tall oil+15 moles ethylene oxide -----    | 15   |
| Aromatic solvent -----                    | 40   |
| Octynol -----                             | 5    |
| Aromatic solvent -----                    | 15   |
| <sup>2</sup> 4-ethyl-1-octyn-3-ol.        |      |

Column 6, Composition 19 should read as follows:

|                                            | Gms. |
|--------------------------------------------|------|
| Composition 11 -----                       | 30   |
| Aromatic solvent -----                     | 50   |
| Octynol <sup>2</sup> -----                 | 10   |
| Nonyl phenol+12 moles ethylene oxide ----- | 10   |
| <sup>2</sup> 4-ethyl-1-octyn-3-ol.         |      |

Signed and sealed this 11th day of January 1972.

(SEAL)  
Attest:

*[Signature]*

EDWARD M.FLETCHER,JR.  
Attesting Officer

ROBERT GOTTSCHALK  
Acting Commissioner of Patents